

## UNITED STATES PATENT OFFICE

2,365,011

## LUBRICANT COMPOSITION

Raphael Rosen, Elizabeth, N. J., assignor to  
 Standard Oil Development Company, a corpora-  
 tion of Delaware

No Drawing. Application September 6, 1941,  
 Serial No. 409,831

2 Claims. (Cl. 252—39)

The present invention relates to improvements in lubricants and especially to the improvements of lubricating oils principally useful for internal combustion engines operating under severe conditions.

Lubricating oils which exhibit improved performance under all types of operating conditions when used for lubrication of heavy duty gasoline engines and for Diesel engines are coming into greater and greater demand. It has been proposed to add various ingredients to these oils to bring about greater engine cleanliness and to avoid ring sticking, varnish formation, sludging, and carbon deposition. It is an object of the present invention to provide addition agents for lubricating oils which will exhibit satisfactory properties of the above type and will at the same time avoid the corrosion of metal parts which often accompanies the use of detergent addition agents.

It is known that, while many metal salts of carboxylic acids, metal alcoholates, metal phenolates, metal enolates, etc., have satisfactory detergent action, these compounds generally have such a corrosive action on the metal parts that their use in internal combustion engines is prohibited. This corrosiveness is apparently due to the formation of oil-soluble organic acids by chemical breakdown of the addition agents during use of the lubricating oils in which they are blended. The additives differ in their corrosive tendency both with respect to the class of compounds and with respect to the metal surfaces involved.

In accordance with the present invention a metallic compound is used which has the detergent properties of the aforementioned metallic salts, but which, if decomposition occurs under the conditions of use, will leave only harmless residues which will not have the corrosive action of such salts. The new addition agent of the present invention is a metallic salt of an organo-carbonic acid, by which is meant a metallic salt of a carbonic acid having one of its hydrogen atoms substituted by an alkyl, aryl, aralkyl, or alkaryl group, or derivatives of these groups, such groups being of sufficient hydrocarbon size to render the compound soluble in mineral lubricating oils. The invention also includes the use of compounds similar to the above in which the metal is attached to the carbonyl group through sulfur, selenium or tellurium, instead of oxygen.

The new class of lubricating oil addition agents of the present invention may be defined in its broadest aspects as the compounds formed from

metals of groups I, II, III, IV, and VIII of the periodic table by joining at least one of the valence bonds of the metals to radicals of the formula



where X is a non-metallic element of group VI of the periodic table, viz., oxygen, sulfur, selenium, or tellurium, and R is an organic radical, including the alkyl, aryl, cycloalkyl, aralkyl, and alkaryl radicals. These radicals may contain various substituent atoms such as oxygen, halogen, sulfur, nitrogen or phosphorus, or substituent groups such as hydroxy, mercapto, amino, alkoxy, aroxy, alkyl or aryl.

When the metal is polyvalent all of its valences may be satisfied with the above type of radical or one or more of them may be connected to other 20 radicals. The metal compounds of the present invention may thus be represented by the general formula



25 in which X and R have the same significance as described above, M is a basic substance, such as a metal or salt-forming group, and T is one or more radicals from the group: carbonate, dithiocarbonate, trithiocarbonate, alkoxy, mercapto, aroxy, thioaroxy, carboxy, thiocarboxy, dithiocarboxy, and the like. The subscript n is an integer whose value is chosen to satisfy valence requirements. When M is monovalent, n is obviously zero. When n is more than one, the 35 groups represented by T may be alike or different.

Among the metals whose salts may be employed in this invention are calcium, barium, magnesium, cadmium, zinc, tin, cobalt, iron, nickel, aluminum, chromium, sodium, lithium, and potassium. Also, 40 it is often advantageous to employ salts of salt-forming groups of non-metallic elements. Thus M in the above formula may also represent ammonium, quaternary ammonium, phosphonium, sulfonium, or pyridonium groups and the like.

The particular compound selected for use will be one which is of sufficient hydrocarbon size to render it appreciably soluble in mineral oils. In general, it is preferred to use compounds having 45 at least ten carbon atoms in the radical R. In some cases the number of carbon atoms may be somewhat less than this, especially when solubilizing groups or atoms, such as chlorine, are introduced into the molecule. Among the particular compositions preferred for use in accordance with

this invention may be mentioned the barium salt of oleyl ester of carbonic acid, the calcium salt of wax alcohol esters of carbonic acid, especially the salt of esters derived from alcohols obtained from paraffin wax, the magnesium salt of sperm oil esters of carbonic acid, the nickel salt of 2,4,5-cumobenzyl carbonic acid, the tin salt of octadecyl ester of monothiocarbonic acid, sodium salt of diisobutyl thiocresol ester of monothiocarbonic acid, and the zinc salt of cyclohexanol ester of monothiocarbonic acid.

The compounds of the present invention may be prepared by methods well known to the art. For example, the metallic salts of alkyl carbonic acids may be prepared by first reacting carbonyl chloride with the desired alcohol to form a chlor-alkyl carbonic acid, as follows:



The latter may then be reacted with a metallic base to form the metallic salt of the alkyl carbonic acid, as follows:



Similar compounds may be formed by reacting a metallic alcoholate with carbon dioxide under pressure as follows:



In this case the alcoholate, if it is derived from a long chain alcohol, is conveniently prepared by reacting a higher alcohol with a metallic alcoholate derived from a low molecular weight alcohol. The corresponding sulfur compounds may be prepared by reacting the proper metallic base with alkyl mercaptan, e. g., lauryl mercaptan, to form the corresponding metallic mercaptide. This mercaptide may be reacted with carbon dioxide to form the metallic salt of thiocarbonic acid, as follows:



Such salts may also be formed by the reaction of a metallic base with a dialkyl dithiocarbonic acid ester  $R_1COCSSR_2$ , where the R's are alkyl groups, as follows:



A further method of preparing the metallic salts of monothiocarbonic acid consists in reacting a metallic alcoholate with carbon oxysulfide, as follows:



Generally, the amount of salt to be used in the lubricant compositions of the present invention should be between the approximate limitations

of 0.02% and 2.0%, and preferably from 0.1% to 1.0%, the exact amount to be used depending to a certain extent on the particular compound, the character of the mineral oil base and the operating conditions of the engine in which the lubricant is to be used.

The lubricating oil base stock for this invention, in its broadest aspect, may be any mineral oil distillate, residual oil or blend and it may be a fraction resulting from various physical and chemical refining treatments, such as solvent extraction, precipitation, etc. For the best results the base stock chosen should usually be that oil which, without the additive present, gives the optimum performance in the service contemplated. For the lubricating of medium and high speed Diesel engines it has been general practice to use a lubricating oil base stock prepared from naphthenic or aromatic crudes and having a Saybolt viscosity at 200° F. of 45 to 90 seconds and a viscosity index of 0 to 50. However, preference is often expressed for oil of very high viscosity index (up to 100 or higher) and such oils may be employed in the present invention. The oils may be free from other addition agents or they may contain other materials for particular purposes, for example, thickeners, sludge dispersing agents, dyes, pour depressants, viscosity index improvers, solvents, coupling agents, oiliness agents, corrosion inhibitors, and antioxidants.

The additives of the present invention are useful in applications other than in mineral oil compositions, particularly as additives for other hydrocarbon base stocks. Thus, they may be added to liquid fuels to increase their wetting ability for metals, enabling them to displace moisture which might otherwise cause corrosion of containers, fuel lines, pump parts and the like. Also they may be added to waxes and asphalt compositions to give improved adhering properties. For similar reasons, the additives may also be employed in greases and other thickened oils.

The present invention is not to be considered as limited by any of the examples described herein which are given by way of illustration only, but it is to be limited solely by the terms of the appended claims.

I claim:

- 50 1. A lubricant comprising a major proportion of a mineral oil base stock and 0.02% to 2.0% of the barium salt of oleyl ester of carbonic acid.
2. A lubricant comprising a major proportion of a mineral oil base stock and 0.2% to 2.0% of a metal salt of the oleyl ester of carbonic acid, the metal of the salt being a metal of group II of the periodic table.

RAPHAEL ROSEN.